

## 1

3,563,793

**FIREPROOFED CELLULOSIC MATERIAL**

Hans Brandeis, Limburgerhof, Pfalz, Klaus Pfleger, Ludwigshafen (Rhine), and Heinz Bille, Limburgerhof, Pfalz, Germany, assignors to Badische Anilin- & Soda-Fabrik Aktiengesellschaft, Ludwigshafen (Rhine), Germany

No Drawing. Filed July 3, 1968, Ser. No. 742,182  
Claims priority, application Germany, July 5, 1967,

P 15 94 937.8

Int. Cl. C09d 5/18; C09k 3/28

U.S. CL. 117—136

4 Claims

**ABSTRACT OF THE DISCLOSURE**

Fireproofing cellulosic fibrous material with compounds having the formula:



in which  $a$  denotes a value from 0.1 to 2.6,  $b$  a value from 0.3 to 2 and  $c$  a value from 0.1 to 1.0 the total of  $a$ ,  $b$  and  $c$  being 3, and cellulosic material fireproofed therewith.

The present invention relates to a process for the fireproofing of cellulosic fibrous material using certain phosphorus amides.

The amides, particularly the dialkylamides and the 1,2-alkylenamides of phosphoric acid are generally known as fireproofing agents for cellulosic fibrous material.

It is possible by means of these agents, which are in general fixed to the fibrous material by heating, to diminish the flammability of the fibrous material considerably, but usually only with impairment of other desirable properties. For example, this treatment may produce brittleness, a tendency to yellow of textiles finished in this way, and low resistance to washing in the case of some of these prior art fireproofing finishes. This is especially true of the compounds giving the fireproofing effects which have hitherto been the best and most resistant to washing, particularly tris-N-aziridinylphosphine oxide (phosphoric acid triethylenimide, APO), which has the formula:



and is very toxic in the unchanged, i.e. unfixed, condition. When using other phosphoric amides (including the non-toxic compound phosphoric-tris-methylamide) good fireproofing effects are obtained, but they are not resistant to washing.

It is known from British patent specification 830,800 that a mixture of approximately equal parts of monoethylenamidophosphoric acid diamide and ammonium chloride may also be used for flameproofing. This substance is however not very suitable for practical use for the reason alone that it contains large amounts of ineffective ammonium chloride which cannot be separated.

The object of the present invention is to provide new and highly effective fireproofing agents for cellulosic fibrous materials which give optimum and wash-resistant fireproofing effects with a minimum of deleterious secondary effects.

We have found that cellulosic fibrous materials can be given a wash-resistant fireproof finish by means of phosphoric amides by applying to the fibrous material

## 2

a composition containing or consisting of a mixture of compounds which is defined by the general Formula I:



in which  $a$  may have any value from 0.1 to 2.6,  $b$  any value from 0.3 to 2.0 and  $c$  any value from 0.1 to 1.0, the total of  $a$ ,  $b$  and  $c$  being 3 and the indices corresponding to the average frequency of the methylamido, ethylenamido and amido groups in weighable amounts of the trivalent compound (I).

The mixtures of compounds (I), which are referred to hereinafter as compounds for simplicity, are obtained by conventional methods, preferably by reaction of 1 mole each of phosphorous oxychloride with  $a$  moles of methylamide,  $b$  moles of ethylenimine and  $c$  moles of ammonia in an inert organic solvent at temperatures of from about  $-40^\circ$  C. to  $+40^\circ$  C. It is recommended that the solvent (for example methylene chloride, benzene, dioxane, tetrahydrofuran or ether) be placed in a reactor and the reactants be passed into the same simultaneously at the same rate in proportion to the molar composition of the product. An appropriate molar excess of a tertiary amine such as trimethylamine or triethylamine should be used to bind hydrogen chloride liberated in the reaction. The hydrochlorides of the tertiary amines are insoluble in the said solvents and can be filtered off therefrom. The solution is then evaporated, advantageously at subatmospheric pressure, after which the product remains as a colorless syrupy liquid. So that it should remain stable for long periods it is advisable to dilute it, for example with dioxane, dimethylformamide or low molecular weight water-soluble alcohols. The mixtures of molecules formed have statistical distribution of the amine radicals on the phosphorus.

By "applying to the fibrous material" we mean using the flameproofing mixture by a conventional method or any method which is known in the art.

The new agents are advantageously used in 5 to 50% aqueous solution (percentage here and hereinafter being by weight) for finishing cellulosic fibrous materials, the amount being such that the fibrous material absorbs from about 5 to 50%, preferably from 10 to 30%, of the dry weight of (I) depending on the desired intensity of the fireproofing effect. Application may be for example by dipping, spraying or padding. After the impregnated fibrous material has been dried, the agent is fixed thereon by heating for from about two to twenty minutes at about  $100^\circ$  to  $200^\circ$  C., preferably from  $150^\circ$  to  $170^\circ$  C. Following this, the fibrous material thus finished is given a conventional after-treatment for removal of unfixed agent; for example it may be washed with hot dilute aqueous alkali metal hydroxide solution or alkali metal carbonate solution.

The agents (I) are compatible with all other agents for textile finishing, particularly with a great variety of aminoplast-forming monomeric, oligomeric and polymeric compounds and may be used together with them. In other respects, the method according to this invention may be carried out by all procedures and in all apparatus which would otherwise be used for finishing fibrous materials.

Cellulosic fibrous materials may include cotton, linen, sisal, hemp, regenerated cellulose and wood-wool in the form of filaments, threads, fibers, wadding, nonwoven fabrics or sheet materials, such as textiles and papers of all types. These materials may be mixed with others, for example wool, silk, polyester, polyamide or polyacrylonitrile, the total fireproofing effect then corresponding more or less to that of the cellulose fraction.

